

March 25, 1969

R. J. BONDLEY

3,434,812

THERMIONIC CATHODE

Filed Sept. 8, 1966



INVENTOR:  
RALPH J. BONDLEY,

BY *James J. Lichello*  
HIS ATTORNEY.

3,434,812

## THERMIONIC CATHODE

Ralph J. Bondley, Scotia, N.Y., assignor to General Electric Company, a corporation of New York  
 Continuation-in-part of application Ser. No. 360,439,  
 Apr. 16, 1964. This application Sept. 8, 1966, Ser.  
 No. 578,060

Int. Cl. B22f 5/00

U.S. Cl. 29—182.5

5 Claims

## ABSTRACT OF THE DISCLOSURE

An improved dispenser cathode having an emission density of the order of 10 a./cm.<sup>2</sup> at 1000° C. consisting essentially of a refractory metal matrix including 5–11% by weight barium-strontium-tungstate  $Ba_5Sr(WO_6)_2$ .

This application is a continuation-in-part application of copending application Ser. No. 360,439 filed Apr. 16, 1964, now abandoned, and assigned to the same assignee as the present invention.

This invention relates to improved dispenser cathodes and more particularly to an improved high emission density thermionic cathode and a prescribed process of combining and activating certain specifically prescribed ingredients to obtain increased high emission density characteristics.

In various electronic applications generally, and particularly with respect to high power output beam devices operative in the ultra high frequency and microwave frequency ranges, a dispenser cathode plays an extremely important if not limiting part for increased power output. Increased power output in many of the frequency generation devices may be obtained by means of thermionic cathodes capable of emitting a stable D-C current of high density over a long period of time with comparatively small heater power consumption. There is an ever increasing need, for example, for hot cathode devices which are capable of operating over many hundreds of hours of continuous operation in the temperature ranges of 900° to 1200° C. and which will, under these conditions, provide an emission current density of in excess of at least 5 amperes per square centimeter. Such a dispenser cathode as described, when employed in a high frequency generator depending upon a high power electron beam, will provide a substantial increase in the power output of the generator in addition to the overall increase of efficiency thereof.

Accordingly, it is an object of this invention to provide an improved thermionic dispenser cathode.

It is another object of this invention to provide an improved process to yield an increased emission density cathode.

It is yet another object of this invention to provide a continuous high emission density from a barium tungstate cathode.

It is a further object of this invention to provide an improved process to provide barium tungstate dispenser cathodes of increased emission densities at lower temperatures under continuous use.

It is another object of this invention to provide an improved thermionic dispenser type cathode comprising a sintered mixture of a refractory metal having interspersed therein a solid solution of a pair of barium compounds, and operative for high emission density at lower temperatures.

It is a further object of this invention to provide an improved sintering and shaping process in the manufacture of barium strontium tungstate and dispenser cathodes.

It is a further object of this invention to provide a

barium strontium tungstate dispenser type cathode for general usage which will have an emission density of in excess of at least about 5 amperes per square centimeter emission density at temperatures below about 1000° C. over extended periods of time.

5 Briefly described, this invention in one of its preferred forms includes the combination of specific proportions of certain powdered ingredients, for example barium carbonate ( $BaCO_3$ ), strontium carbonate ( $SrCO_3$ ), and tungsten trioxide ( $WO_3$ ), which are intimately mixed, wet milled, dried, and fired in pellet form to provide a solid solution of barium compounds such as  $Ba_3WO_6$  and  $Ba_2SrWO_6$  in generally equal amounts. The pellets are then crushed and sieved, and about 9% by weight thereof is mixed with about 1% by weight zirconium hydride and about 90% by weight tungsten metal powder. The resulting mixture is dry milled, compacted under high pressure, and then subjected to high temperatures in a reducing atmosphere to fuse or melt one of the barium compounds and provide an integral cohesive body which is formed as a high current density thermionic dispenser type cathode.

10 This invention will be more fully understood when taken in connection with the following description and the drawing in which:

15 The figure is an exemplary illustration of an assembly utilizing a dispenser cathode of this invention.

20 In the dispenser cathode prior art there exists a vast number of different processes potentially employing the same materials, which in turn provide different dispenser cathodes. By the same token the dispenser cathode prior art indicates a great number of various ingredients and various proportions and mixings thereof which in turn provide different dispenser cathode characteristics. In 25 many of these instances the intermediate reaction and combinations which take place in the production of a dispenser cathode are not known, and at the same time, in a great number of instances those ingredients originally employed to provide the cathode do not appear in the final cathode in the same form or in the same amount. Therefore, it is not readily apparent by examination just what specific material, or combinations of materials, or process steps give rise to a preferred cathode, or which 30 parameters may provide a greatly increased emission density.

35 The prior art of dispenser cathodes is indicative of barium tungstate cathodes representing a potential area from which dispenser cathodes of substantially increased continuous emission densities at low temperatures might

40 be obtained. It has been discovered that a barium tungstate thermionic cathode having the constituents above described, and in the proportions given, provides a very high emission density disproportionate to the known reaction or contributions of the constituent elements. In addition, 45 this very high emission density takes place at lower temperatures and is continuous for long life operation. Such cathodes may be produced repetitively in large numbers by following certain prescribed proportions and process steps.

45 It has also been discovered in this invention that critical items with respect to a high emission density cathode are related as well as to those ingredients appearing in the final item as to the beginning ingredients. In addition, certain final processing may change or alter 50 the original ingredients to provide the final ingredients in a more desired form sometimes irrespective of the particular amount of particular material available in the original form.

55 The basic dispenser cathode of this invention includes a porous matrix metal body having therein a tungstate activator material and a reducing agent. The matrix body

is a refractory metal, for example one or more of those metals taken from Groups IV, V and VI of the Periodic Table of Elements such as tungsten, molybdenum, rhenium, tantalum, etcetera, and in a preferred form of this invention is tungsten. The matrix body is further defined as composed of a starting material which is finely divided or powdered high purity tungsten preferably having an average particle size in the range of about 2-5 microns. Particle sizes in excess of this range provide less than optimum results in the final product as based upon a series of exemplary cathodes of varying tungsten matrix particle sizes. Powdered refractory metals, particularly tungsten, have been employed in this invention in a general range of from about 80 weight percent to about 94 weight percent. A preferred range is from about 88 weight percent to about 92 weight percent with best results from about 90 weight percent to about 92 weight percent.

The activator material which is included in the matrix material is a barium tungstate compound, which, under operative conditions of the cathode, will be reduced and dispense barium to an active surface of the cathode. One or more barium compounds may be so employed. It has been discovered that best results are obtained in the practice of this invention when the activator starting material includes a single phase solid solution of equimolecular amounts of  $\text{Ba}_3\text{WO}_6$  and  $\text{Ba}_2\text{SrWO}_6$  having cubic symmetry. Peak emission density at lower temperatures is obtained when the noted barium-strontium compounds are provided in substantially stoichiometric proportions. The strontium containing tungstate has been found superior to other alkaline metal tungstates. Other barium compounds which may be employed as activator materials are  $\text{BaO}$ ,  $\text{Ba}_2\text{CaWO}_6$ , etcetera, which may provide tailored cathodes for specific usage where maximum density proportionate to lower temperature and longer life is not the major circumstance. The activator material has been employed in this invention in the general range of from about 5 weight percent to about 11 weight percent with from about 7 weight percent to about 9 weight percent being a preferred range.

The reducer material employed in the dispenser cathode of this invention performs the function of reducing the barium compound so that barium may migrate through the porous tungsten body to provide an active low work function surface. While there are various materials, elements or compounds which may be added to the cathode to provide this function, it has been discovered that only a limited number of refractory metals provide optimum results. Zirconium is one preferred reducer metal in the practice of this invention. Zirconium should be added by way of a zirconium compound such as a hydride, zirconate or oxide. Zirconium hydride,  $\text{ZrH}_2$ , as a preferred compound provides distinguishable results by emission density tests over the other reducer compounds. Zirconium hydride has been employed in this invention in the general range of at least a significant amount, i.e., an amount which will provide measurable reduction to about 2.5 weight percent with a preferred range being from about .25 weight percent to about 1.0 weight percent. Incremental additions of  $\text{ZrH}_2$  to standardized mixes of matrix metal and activator compound indicate, by emission tests, that negligible improvement is obtained by greater amounts, and particularly, diminishing results are noted in many instances.

It has also been discovered that hafnium may be employed as a reducer metal in this invention. Hafnium may be added by way of such compounds as oxides and hydrides, hafnium hydride  $\text{HfH}_2$ , being preferred in proportions which may include up to about 2 weight percent. The amount of hafnium to be added should also be maintained in the same general range as expressed for  $\text{ZrH}_2$ , taking into consideration the different atomic weight involved. Other refractory metals, particularly titanium, may be employed but with distinguishable diminishing and non-equivalent results.

In the preparation of the initial materials, very great importance is attached to proportions, particle sizes, mixing time, compression pressures, firing or sintering temperatures and other related parameters, with respect to the final emission properties and life of a cathode. It is a common occurrence to seriously alter an otherwise optimum cathode by an inadvertent or mistaken or incorrect change of materials or processes or by assuming an equivalency not borne out by experimentation.

It has been discovered that one outstanding and preferred cathode of this invention, i.e., one having a long life with a substantially continuous emission density of about 10 amperes/cm.<sup>2</sup> at a temperature below about 1000° C., is provided in the specific controlled proportions of ingredients. For example, these ingredients may comprise a general range of 88% to 92% by weight of refractory metal, about 7% to 9% by weight barium compound and the balance, usually about 0.25 to 2.5% by weight of a reducer material. For a high emission density cathode approaching 10 or more amperes per square centimeter at 1000° C. or less, a more preferred range, and materials, are about 90% to 92% by weight tungsten, 7% to 9% by weight of a single phase solid solution corresponding to the general formula  $\text{Ba}_5\text{Sr}(\text{WO}_6)_2$  obtained by a reaction of constituents such as for example  $\text{Ba}_3\text{WO}_6$  and  $\text{Ba}_2\text{SrWO}_6$ , and from about 0.5% to 1.0% zirconium hydride. Outstanding examples include

(a) about 92% by weight tungsten, about 7½ by weight of the described solid solution activator compound and about 0.5% by weight zirconium hydride, and  
 (b) about 90.2% by weight tungsten, about 9.2% by weight activator compound as described, and the balance zirconium hydride, about 0.6% by weight.

The proportions so indicated may be further described by a major percent by weight of refractory metal, i.e., 50 weight percent or more, a minor percent by weight of an activator material, i.e., less than 50% by weight, and an additive but significant amount of a reducer material which is substantially less than the amount of activator material.

The process requirements of cathodes made in accordance with the proportions above indicated are critical to the emission density characteristics of the final dispenser cathode. Best results are obtained when considerable care is exercised to maintain cleanliness in conjunction with the use of high purity materials. In a preferred form of this invention, the activator material is provided by wet milling in methanol a combination of barium carbonate

( $\text{BaCO}_3$ )  
 strontium carbonate ( $\text{SrCO}_3$ ), and tungsten trioxide  
 ( $\text{WO}_3$ )

in substantially stoichiometric proportions. After milling sufficiently to provide a very intimate mixture, the methanol is decanted and the powder material is dried and compressed into pellets in a hydraulic press. These pellets are thereafter fired in an air or oxygen atmosphere at a temperature above 1400° C. for several hours.

X-ray analysis of these pellets indicates a solid solution of  $\text{Ba}_3\text{WO}_6$  and  $\text{Ba}_2\text{SrWO}_6$  at a composition of 50 atomic percent. Best results have been obtained with this composition. However, variations are tolerable for a number of specific applications where criteria other than or in addition to high emission rate is required. The 50 atomic percent composition depends on the ratio of starting materials particularly for example a ratio in stoichiometric proportion such as 18.525 grams  $\text{BaCO}_3$  barium carbonate, 2.770 grams  $\text{SrCO}_3$  strontium carbonate and 8.705 grams  $\text{WO}_3$  tungsten oxide. The reaction product is

$\text{Ba}_5\text{Sr}(\text{WO}_6)_2$   
 or alternately 5 $\text{BaO} \cdot \text{SrO} \cdot 2\text{WO}_3$ .  
 After firing the pellets are crushed and sieved through

a 325 mesh screen. This material is then mixed with tungsten which is provided in finely divided or powder form with an average particle size of 2-5 microns. The proportions are in the ranges previously described, particularly specific examples (a) and (b). To this mixture there is added a reducer such as zirconium hydride or hafnium hydride also of about 325 mesh or finer particle sizes, also in the preferred range given, specific examples being by weight,  $\frac{1}{2}\%$  and 0.6% respectively. This mixture is then placed in a mixing apparatus, in this instance a small molybdenum ball mill, and milled for several hours. The milling time for optimum emission is a function of the mill size, speed and charge for one particular mill.

In operative practices of this invention, ball milling was performed in an all molybdenum ball mill. The mill chamber was in the form of a molybdenum cup measuring about  $2\frac{3}{4}$  inches diameter and  $2\frac{3}{4}$  inches depth. The milling or grinding members were molybdenum slugs of about  $\frac{1}{4}$  inch diameter and  $\frac{1}{4}$  inch length. Fifty of these milling members were employed for each milling session or operation. A molybdenum cover plate was secured to the open end of the mill chamber during a milling operation. During operation the mill revolved at the rate of 120 r.p.m.

Operative curves, i.e., emission density vs. milling time, of a representative number of these milling operations indicated a peak condition of emission in the 2 to 6 hour milling operation range. Unexpectedly it was discovered that in extended milling operations a second emission peak occurred in the 12 to 18 hour range. Best emission results were obtained in cathodes of this invention when the second peak condition was utilized, i.e., where ball milling of the constituents was continued for 12 to 18 hours.

After milling, the powder mixture is then placed in a die and compacted in a hydraulic press into pellets of the general desired size. Compacting pressures contribute to the final characteristics because they predetermine to some extent the pore size of the finished product. In the practice of this invention compacting pressures were employed in the range of about 40 to 90 tons/in.<sup>2</sup>. Between about 80 to 90 tons/in.<sup>2</sup> provided best results.

The pressed powder pellets were sintered by heating in a predetermined atmosphere at about 1900° C. for a period of a few minutes to about 5 or 6 minutes. Sintering is carried out under a relatively high purity reducing atmosphere. For example, a high purity hydrogen atmosphere which was carefully deoxygenated and dried was employed in the preferred practice of this invention. It was noted that the presence of contaminants in the hydrogen, for example water vapor and other gases, markedly affected the emission characteristics of the final cathode by reducing obtainable emission densities. The hydrogen employed had a dew point below about -100° F. It was further noted that the final product from hydrogen sintering was superior to those cathodes sintered under other atmospheres, such as inert gas atmospheres, or other atmospheres consisting of a mixture of hydrogen and an inert gas. Additionally, comparative emission density results indicate that the sintering process should be carried out at temperatures in excess of about 1800° C. with optimum results falling between 1850° and 1900° C., which is at or above the melting point of  $\text{Ba}_3\text{WO}_6$ , higher temperatures not indicating any further favorable results.

After sintering, the cathode bodies are prepared by having the emitting surface suitably formed or shaped to provide a fresh active surface, generally by a clean removal of a thin layer of the cathode. Best results were achieved when a cathode surface was carefully lathe machine with the use of a very sharp Carboloy cutting tool similar to a facing tool. A high head stock speed, thin and slow cross feed cut is employed. It is believed that this type of cutting process exposes and/or prepares an optimum surface with excellent communication into the porous body. The pore openings of the surface are not deformed or

closed by this process. Other similar processes include sputtering or electron machining. Comparative results indicate a markedly superior cathode is provided by the machining or cutting process as compared to, for example, an uncut surface or one obtained by grinding by different abrasive wheels, i.e., diamond or alundum wheels.

A great number of dispenser cathodes have been produced by the described process. These dispenser cathodes provided greatly increased emission densities at low temperatures for continuous operation, unexpected in view of the prior art knowledge of dispenser cathode technology. Emission density measurements were carried out in a manner to substantially preclude any errors in the test equipment and to provide a measurement more reliable and precise than those indicated in ASTM standardization test diodes for cathode evaluation. In this connection a vacuum system was constructed from 347 stainless steel and bakable to the extent of freeing the system from water vapor or absorbed gases. All openings were made through metal ceramic seals and compression flanges. The system is initially pumped by mercury diffusion pump because mercury is a well defined substance that does not break down or decompose with heat and is not deleterious to cathode emission. For the higher evacuation conditions an ion pump was utilized to bring the pressure of the system to about  $10^{-7}$  torr. A cathode diameter of one centimeter was chosen as being representative of sizes encountered in microwave tubes. Since cathodes of this size and made in accordance with this invention are capable of delivering large currents, a six-phase variable voltage rectifier of 20 amperes capacity at 500 volts was constructed and used for all measurements. The ripple encountered in six-phase rectification is low enough to permit the RMS values to be equivalent to straight D-C measurements. Anode dissipation is one of the first problems encountered in high current measurements. To keep anode dissipation to a minimum, diodes with 0.010 inch anode-to-cathode spacing were chosen as being a well defined compromise of electrical and mechanical considerations. Even with these close spacings, power densities of about four to six kilowatts per square centimeter are encountered at current levels approaching 10 amperes. These are near maximum power concentrations that can be dissipated with water-cooled anodes.

A substantial number of cathodes in accordance with the practice of this invention were produced to better determine and define optimum materials, material proportions, process step times and other parameters. For example, in representative numbers of cathodes with all other parameters being maintained equal, both the kind and the proportion of given materials were varied, as well as process steps. For each change emission density measurements were taken to indicate the effect of the change. Among these changes are included proportional change of materials, the use of other refractory metals such as molybdenum and combinations thereof, the use of other additive materials and other alkaline earth activator compounds, the use of other sintering atmospheres, and the use of other active surface preparation means. The results of these investigations reveal that preferred cathodes are those containing

- (a) about 92 weight percent tungsten, about  $7\frac{1}{2}$  weight percent barium compound which includes a solid solution of  $\text{Ba}_3\text{WO}_6$  and  $\text{Ba}_2\text{SrWO}_6$  and about  $\frac{1}{2}$  weight percent  $\text{ZrH}_2$  and
- (b) 90.2 weight percent tungsten, 9.2 weight percent solid solution and the balance zirconium or hafnium hydride.

Furthermore, using the standard optimum proportions above described, process steps were varied over a wide range and emission densities of the resulting cathodes compared. The results reveal that the most preferred cathode includes the solid solution of  $\text{Ba}_3\text{WO}_6$  and  $\text{Ba}_2\text{SrWO}_6$  in the activator material, sintering in a high purity re-

ducing (hydrogen) atmosphere and very sharp clean cutting preparation of an emitting surface.

Repetitive cathodes are accordingly produced by this invention having continuous emission densities in excess of 7 to 10 amperes per square centimeter at operating temperatures from about 850 to 1000° C. when the preferred compositions and production parameters as described are followed.

The dispenser cathodes of this invention may be utilized in a number of different assemblies and configurations. A common example 10 is illustrated in FIG. 1. In FIG. 1 a generally cylindrical button or pill 11 of the dispenser cathode of this invention is concentrically fixed or contained within the end of a support cylinder 12. Button 11 is provided with an exposed emitting face surface 13 and an opposite surface 14 which is adjacent a filamentary type electrical heater 15. Button 11 may be a separate assembly which is joined to cylinder 12 or may be formed therein in position. Cylinder 12 is preferably a refractory material for example molybdenum, 20 tungsten, et cetera.

While this invention has been described with reference to particular and exemplary embodiments thereof, it is to be understood that numerous changes can be made by those skilled in the art without actually departing from the invention as disclosed, and it is intended that the appended claims include all such equivalent variations as come within the true spirit and scope of the foregoing disclosure.

What is claimed as new and desired to be secured by 30 Letters Patent of the United States is:

1. A thermionic cathode composition consisting essentially of an intimate mixture of

- (a) from about 88% to 94% by weight of finely divided refractory matrix metal,
- (b) from about 5% to 11% by weight of a solid solution consisting of 50 atomic percent  $Ba_3WO_6$  and 50 atomic percent  $Ba_2SrWO_6$ , and
- (c) from about 0.25% to 2.5% of a refractory metal reducer material.

2. A thermionic dispenser cathode composition consisting essentially of an intimate mixture of

- (a) at least about 90% by weight of refractory in a finely divided form of from about 2 to 5 microns average particle size,
- (b) at least about 7.5% by weight of a solid solution

consisting of 50 atomic percent  $Ba_3WO_6$  and 50 atomic percent  $Ba_2SrWO_6$ , and

(c) at least a small but effective amount of a refractory metal reducer material.

5 3. The invention as recited in claim 2 wherein said refractory metal is tungsten and said refractory metal reducer material is zirconium.

4. As an article of manufacture a sintered integral cohesive thermionic dispenser cathode consisting essentially of

- (a) 88 to 94 percent by weight of a porous refractory metal matrix body,
- (b) 5 to 11 percent by weight of a single phase barium-strontium-tungstate crystal of a composition corresponding to the general formula  $Ba_5Sr(WO_6)_2$ , and
- (c) 0.25 to about 2.5 weight percent of a further refractory metal throughout said cathode as a reducer material for said barium-strontium-tungstate at operative cathode temperatures,
- (d) said cathode having a useful emission current density in excess of 5 amperes per square centimeter at 1000° C. of continuous operation.

5. As an article of manufacture of thermionic dispenser cathode consisting essentially of

- (a) a sintered powdered tungsten body of average particle size of from 1 to 5 microns which comprises from about 88% to 94% by weight of said cathode,
- (b) about 7.5% by weight of a single phase solid solution consisting of 50 atomic percent  $Ba_3WO_6$  and 50 atomic percent  $Ba_2SrWO_6$  dispersed throughout said cathode, and
- (c) 0.25 to 1% by weight of zirconium distributed throughout said cathode as a reducer.

#### References Cited

##### UNITED STATES PATENTS

- |           |        |                |       |          |
|-----------|--------|----------------|-------|----------|
| 2,848,644 | 8/1958 | Koppius        | ----- | 313—346  |
| 2,881,512 | 4/1959 | Huber et al.   | ----- | 29—182.5 |
| 3,269,804 | 8/1966 | Affleck et al. | ----- | 29—182.5 |

LELAND A. SEBASTIAN, Primary Examiner.

A. J. STEINER, Assistant Examiner.

U.S. CL. X.R.

45 313—346